

# UNITED STATES PATENT OFFICE.

ANSEL C. DENNING, OF JOHNSON CITY, NEW YORK.

## FELTED MATERIAL AND PROCESS OF MAKING SAME.

1,377,007.

Specification of Letters Patent.

Patented May 3, 1921.

No Drawing.

Application filed March 16, 1920. Serial No. 366,400.

To all whom it may concern:

Be it known that I, ANSEL C. DENNING, a citizen of the United States, residing at Johnson City, New York, have invented certain new and useful Improvements in Felted Material and Processes of Making Same, of which the following is a clear, full, and exact description.

This invention relates to a felted material and to a process of making such material, and particularly to a felted material that is especially useful for the making of box toes of boots and shoes.

In the manufacture of boots and shoes it is now a common practice to form the box toes of the shoes from felt impregnated with a thermoplastic binder of such a character that the material may be made plastic and pliable by heating, as with steam, whereby it may be shaped to the toe of the last or the toe mold, the material setting to shape when it cools. Before the development of my substitutes for the material heretofore used, such box toes were formed from a wool felt impregnated with a thermoplastic binder.

In my Letters Patent #1,303,262, granted May 13, 1919, I have disclosed a substitute material for making box toes for shoes which can be used in place of the wool felt employed before the said invention and which has been extensively so used, and a general object of the present invention is to provide an improved substitute material of the general character of that disclosed in said Letters Patent, and to provide an improved process for making such materials.

More particularly, the invention aims to provide a felted material for the uses for which such materials are particularly intended, and especially for use in the forming of box toes for shoes, which will have the desirable characteristics of a felt for such uses, among which are capacity readily to absorb the thermoplastic binder, strength to resist the strains and rough usage incident to the lasting operation in shoe making, particularly in the lasting of welt shoes, in which operation it is now the common practice to secure the toe in lasted position by means of a toe wire instead of tacks; and lastly, the capacity to stretch and adapt itself to the curvature of the toe of the last or of the toe mold.

In carrying out my invention I effect a mixture of cotton fibers, wool and tannery hair in such proportions as to produce a

felt having all the various desirable characteristics above set forth, and to obtain this mixture I utilize what have heretofore been largely by-products and frequently 60 waste, the cotton fiber being obtained by treating textile cotton rags in such manner as to reduce the rags to a pulp, the wool being likewise obtained from rags, and the hair being added to the mixture after the 65 wool and cotton rags have been reduced to a pulp.

The following treatment of the constituent materials, mixed in the proportions hereinafter set forth, produces a felted material 70 having all of the desirable characteristics hereinabove mentioned.

Ordinary cotton and woolen textile rags are put into a beater—such, for example, as the ordinary beater or beating engine used 75 in the manufacture of paper—and after the material has been washed clean in the beater, it is beaten until thoroughly disintegrated and until the fibers are quite thoroughly separated, and then the tannery 80 hair is added. The beating action is continued after the addition of the tannery hair until the hair is thoroughly intermixed with the cotton and woolen fibers, after which the material is allowed to discharge into a 85 vat, and from this vat the mixture is pumped onto a sheet-forming screen, such for example as the ordinary cylinder wet machine, where the sheet is formed in a manner very similar to the ordinary operation 90 of paper making. Driers are preferably so arranged as to dry this material continuously.

The following proportions of the materials entering into the composition have 95 been found to impart to the felted material the desired characteristics, to wit, about 40% of cotton rags, 20% of mixed rags, which are largely woolen, and 40% of tannery hair, the wool in such a mixture approximating about 12% of the whole mixture.

The advantage of using a small percentage of wool in a composition of this character is that the wool tends to open up the 105 felt slightly because of its being curled and thus tends to increase the absorbent capacity of the resultant felt and at the same time to facilitate its stretching, the tannery hair coöoperating with the wool to give the material the capacity to stretch and conform to 110 the shape of the toe.

- It is important that the tannery hair be added to the mixture after the textile rags have been substantially reduced to a pulp, in order that the hair itself may not be broken up and thus not play its proper part in the completed felt, this part, as hereinabove suggested, being important in a material intended particularly for use in the making of box toes for shoes.
- 10 After the material has been formed into sheets and dried, it is impregnated with the thermoplastic binder. Such a binder may be formed from a mixture of rosin and asphaltum, and the impregnation of the felt may be effected by forcing the sheet through a hot mixture of the rosin and asphaltum.
- 15 After the impregnated felt has been cooled so that the binder has set, the box toe blanks may be died out and skived on the edges and thus made ready for insertion in the toes, where they are later usually heated by steam and made plastic as hereinabove pointed out.
- 20 It will be understood, of course, that the invention is not restricted to the exact proportions of materials above set forth in the description of an illustrative mixture that has produced satisfactory results, and that its utility is not necessarily restricted to the provision of material for making box toes of shoes.
- 25 What I claim as new is:
1. A felted material of the character described, composed of cotton and woolen rags and tannery hair, the proportion of cotton and of tannery hair being each greater than the proportion of wool in the resultant material.
  2. A felted material of the character described, composed of cotton and woolen tex-

tile rags and tannery hair, the proportion of wool being less than one-half of that of either of the other component materials.

3. A felted material of the character described, composed of cotton, wool and tannery hair, the wool being much less in proportion than either the cotton or the tannery hair.

4. The process of making a felted material of the character described, which consists in forming a mixture consisting of about 40% of cotton textile rags and 20% of mixed cotton and woolen textile rags, and after reducing said rags to a pulp in which the fibers are substantially separated adding to such mixture about 40% of tannery hair, thoroughly mixing said tannery hair with said rag pulp, and then forming a sheet from said pulpy mixture.

5. The process of producing a felted material for use in making box toes of shoes, which consists in reducing mixed textile rags to a pulp substantially such as is employed in the making of paper, adding thereto and thoroughly mixing therewith, while in the pulpy condition, tannery hair, the components of the mixture being in such proportions that the resultant material will contain about 40% of tannery hair and about 12% of wool, and that the remainder shall be substantially all cotton, forming a sheet from said mixture, drying and then impregnating said sheet with a thermoplastic binder.

Signed at Johnson City, N. Y., this 12th day of March, 1920.

ANSEL C. DENNING.

Witnesses:

A. G. CRIMMINS,  
M. B. CAMPBELL.